# EUROPEAN PATENT SPECIFICATION

(11) **EP 1 260 649 B1**
(45) Date of publication and mention of the grant of the patent: **16.07.2008**
(21) Application number: 02011469.0
(22) Date of filing: 24.05.2002
(51) Int. Cl.: E04D 1/20, E04D 1/22, E04D 1/26

(54) **Composite shingle**
Kompositschindel
Bardeau composite

(30) Priority: 25.05.2001 US 865403
(43) Date of publication of application: 27.11.2002
(73) Proprietor: Epoch Composite Products, Inc., Joplin, MO 64801 (US)
(72) Inventor: Jolitz, Randal J., Joplin, Missouri 64801 (US)
(74) Representative: Dehmel, Albrecht

(56) References cited:
- US-A- 4 307 552
- US-A- 5 615 523
- US-A- 6 164 034

## Description

### BACKGROUND

### FIELD OF THE INVENTION

The present invention relates to roofing shingles. Specifically, the present invention relates to composite roofing shingles composed primarily or exclusively of a polyolefin polymer and a filler.

### BACKGROUND OF THE INVENTION

Traditional roofing products include asphalt shingles, wood shakes, slates, and metal panels. Each of these products has benefits. For instance, wood shakes and slate roofing are very aesthetic. However, wood shakes are considered a fire hazard and slate is very expensive and subject to cracking.

Less expensive roofing products have been introduced to simulate wood shakes and slate roofing. Some asphalt shingles have been developed that resemble slate or shake roofing. However, asphalt products typically do not have the structural rigidity of slate or shake. Metal and plastic shingles have been developed that simulate shake and slate. However, those products are subject to denting and breakage.

Composite shingles are typically composed of an organic/polymer component and a filler component see for example US 4 307 552 A. The composition may be molded to simulate the shape and appearance of various types of roofing including shakes or slates. The amount of polymer in these composite shingles is substantially less than the amount of filler. For instance, U.S. patent No. 5,711,126 discloses that the amount of polymer in the composite to range from 12 to 35 % and the preferred amount of filler ranges from 65 to 88%.

Although these composite shingles are capable roofing systems, there are some problems. For instance, the large amount of filler causes the product to be excessively heavy while the low amount of polymer reduces flexibility and increases the possibility of cracking and splitting. Accordingly, a need exists to improve composite shingles.

### SUMMARY OF THE INVENTION

The present invention comprises a composite roofing shingle composed primarily of a mixture of a polyolefin based polymer composition and a filler. The blend includes 70 - 35% polymer and 30 - 65% filler. The preferred mineral is crushed limestone and the preferred polymer is polyethylene. The shingles may be molded to simulate the appearance of traditional roofing or any other configuration that may be advantageous for a particular roofing application.

### DESCRIPTION OF PREFERRED EMBODIMENT

The preferred shingles are composed of a mixture including a polymer and an inorganic. Colorants and other additives may be used to improve or alter the aesthetics or performance of the shingles. Nevertheless, the preferred composition includes a polyolefin and an inorganic filler.

The polymer component is a polyolefin such as polyethelene, polypropelene or mixture of polyolefin polymers. Preferably, this component is polyethelene. The preferred range of this component is 35 to 70% of the composition by weight.

The filler material may include any number or combinations of materials. The preferred filler is an inorganic material such as sand, talc, mica, slate, shale, limestone or fly, volcanic or bottom ash. The preferred filler is crushed limestone. Use of various materials can affect the resulting color of the shingle so selection of the filler can reduce the need for a colorant.

The preferred composition includes a mixture of between 35 to 65% of the polymer component and 65-30% filler component. That mixture provides a lower weight and/or more flexible composite shingle. The preferred composition includes 60% crushed limestone and 40% polyethylene by weight.

The preferred roofing material is made by blending crushed limestone with polyethylene beads or pellets. The mixture is first fed into a mixer, preferably a kinetic mixer. The mixer not only blends the materials but also heats the material to a preferred state where the plastic encapsulates the filler. Color or other additives may be added at this stage. Once the material is mixed, it is conveyed to a piston type extruder and extruded out in shots. A typical shot will weigh between 30 and 35 pounds.

The blend is extruded onto the bottom platen of a mold. Once the material fills the bottom platen of the mold, the top platen of the mold is closed. Pressure is then applied to the top platen to compress the material to fill the entire mold. The preferred mold will be configured to have the shape of wood shakes, or the surface of slate. The preferred mold is approximately 16 feet by 12 inches. The material is cooled to form a board. That board is then cut to length and bundled in different sizes to be shipped.

The shape including the width, thickness contour and length of the shingle may be altered depending on the application. The preferred shingle will be .25 inches thick, 5 inches wide and 12 inches long, where one side is molded to stimulate shake or slate. Color may be added to the mixture during processing or added later.

## Claims

1. A method of applying a composite roofing shingle to a roof, the method comprising the steps of:
a) obtaining a composite roofing shingle consisting of 35 to 65% polyethylene by weight, 30 to 64% inorganic filler by weight, and a colorant ; and
b) applying the composite roofing shingle to a roof.

2. The method of claim 1, where the inorganic filler is crushed limestone.

3. The method of claim 1, where the inorganic filler is slate.

4. The method of claim 1, where the inorganic filler is shale.

5. The method of claim 1, where the composite roofing shingle is configured to have the shape of a wood shake.

6. The method of claim 1, where the composite roofing shingle is configured to have the shape of slate.

7. The method of claim 1, where the composite roofing shingle has one side that has been molded to simulate wood shake.

8. The method of claim 1, where the composite roofing shingle has one side that has been molded to simulate slate.

9. The method of claim 1, where the composite roofing shingle is: less than an inch thick, between about 3-12 inches wide, and between about 6-24 inches long.

10. A method of creating a composite roofing shingle, the method comprising the steps of:
a) creating a composite roofing shingle that includes 36 to 64% polyethylene by weight, and 36 to 64% inorganic filler by weight;
the creating including the steps of:
b) blending the inorganic filler with polyethylene in a mixer; and
c) heating the inorganic filler and polyethylene in the mixer to a state at which the polyethylene encapsulates the inorganic filler.

11. The method of claim 10, where the inorganic filler is crushed limestone.

12. The method of claim 10, where the inorganic filler is slate.

13. The method of claim 10, where the inorganic filler is shale.

14. The method of claim 10, where the creating also includes:
molding at least one side of the composite roofing shingle to simulate wood shake.

15. The method of claim 10, where the creating also includes:
molding at least one side of the composite roofing shingle to simulate slate.

16. The method of claim 10, where the composite roofing shingle is: less than an inch thick, between about 3-12 inches wide, and between about 6-24 inches long.

## Patentansprüche

1. Ein Verfahren zum Anbringen einer Komposit-Dachschindel auf ein Dach, wobei das Verfahren die folgenden Schritte umfasst:
a) das Erhalten einer Komposit-Dachschindel bestehend aus 35 bis 65 Gew.-% der Polyethylen, aus 30 bis 64 Gew.-% anorganischem Füllstoff, und aus einem Farbmittel; und
b) das Anbringen der Komposit-Dachschindel auf ein Dach.

2. Das Verfahren nach Anspruch 1, wobei der anorganische Füllstoff gemahlener Kalkstein (limestone) ist.

3. Das Verfahren nach Anspruch 1, wobei der anorganische Füllstoff Schieferstein (slate) ist.

4. Das Verfahren nach Anspruch 1, wobei der anorganische Füllstoff Schieferton (shale) ist.

5. Das Verfahren nach Anspruch 1, wobei die Komposit-Dachschindel nach einer Holzschindel-Form gestaltet ist.

6. Das Verfahren nach Anspruch 1, wobei die Komposit-Dachschindel nach einer Schieferstein-Form gestaltet ist.

7. Das Verfahren nach Anspruch 1, wobei die Komposit-Dachschindel eine Seite hat, die so geformt wurde, dass sie eine Holzschindel nachahmt.

8. Das Verfahren nach Anspruch 1, wobei die Komposit-Dachschindel eine Seite hat, die so geformt wurde, dass sie einen Schieferstein nachahmt.

9. Das Verfahren nach Anspruch 1, wobei die Komposit-Dachschindel: weniger als ein Inch dick, ungefähr zwischen 3-12 Inch breit, und ungefähr zwischen 6-24 Inch lang ist.

10. Ein Verfahren zum Herstellen einer Komposit-Dachschindel, wobei das Verfahren die folgenden Schritte umfasst:
a) das Herstellen einer Komposit-Dachschindel, die 36 bis 64 Gew.-% Polyethylen, und 36 bis 64 Gew.-% anorganischen Füllstoff beinhaltet;
wobei das Herstellen die folgenden Schritte beinhaltet:
b) das Mischen des anorganischen Füllstoffs mit Polyethylen in einem Mixer; und
c) das Erhitzen des anorganischen Füllstoffs und des Polyethylens in dem Mixer bis zu einem Zustand bei dem das Polyethylen den anorganischen Füllstoff einkapselt.

11. Das Verfahren nach Anspruch 10, wobei der anorganische Füllstoff gemahlener Kalkstein (limestone) ist.

12. Das Verfahren nach Anspruch 10, wobei der anorganische Füllstoff Schieferstein (slate) ist.

13. Das Verfahren nach Anspruch 10, wobei der anorganische Füllstoff Schieferton (shale) ist.

14. Das Verfahren nach Anspruch 10, wobei das Herstellen auch:
das Formen von zumindest einer Seite der Komposit-Dachschindel beinhaltet, um eine Holzschindel nachzuahmen.

15. Das Verfahren nach Anspruch 10, wobei das Herstellen auch:
das Schmelzen von zumindest einer Seite der Komposit-Dachschindel beinhaltet, um eine Schieferschindel nachzuahmen.

16. Das Verfahren nach Anspruch 10, wobei die Komposit-Dachschindel: weniger als ein Inch dick, ungefähr zwischen 3-12 Inch breit, und ungefähr zwischen 6-24 Inch lang ist.

## Revendications

1. Procédé d'application d'un bardeau de toiture composite sur un toit, ledit procédé comprenant les étapes consistant à :
a) obtenir un bardeau de toiture composite constitué de 35 à 65 % en poids de polyéthylène, 30 à 64 % en poids de charge inorganique et d'un colorant ; et
b) appliquer le bardeau de toiture composite sur un toit.

2. Procédé selon la revendication 1, où la charge inorganique est le calcaire broyé.

3. Procédé selon la revendication 1, où la charge inorganique est l'ardoise.

4. Procédé selon la revendication 1, où la charge inorganique est le schiste.

5. Procédé selon la revendication 1, où le bardeau de toiture composite est configuré pour avoir la forme d'un tavaillon.

6. Procédé selon la revendication 1, où le bardeau de toiture composite est configuré pour avoir la forme d'une ardoise.

7. Procédé selon la revendication 1, où le bardeau de toiture composite a une face qui a été moulée pour simuler un tavaillon.

8. Procédé selon la revendication 1, où le bardeau de toiture composite a une face qui a été moulée pour simuler une ardoise.

9. Procédé selon la revendication 1, où le bardeau de toiture composite a une épaisseur inférieure à un pouce, a une largeur entre environ 3 et 12 pouces, et a une longueur entre environ 6 et 24 pouces.

10. Procédé de création d'un bardeau de toiture composite, ledit procédé comprenant les étapes consistant à :
a) créer un bardeau de toiture composite qui comprend de 36 à 64 % en poids de polyéthylène et 36 à 64 % en poids de charge inorganique ;
la création comprenant les étapes consistant à :
b) mélanger la charge inorganique avec le polyéthylène dans un mélangeur ; et
c) chauffer la charge inorganique et le polyéthylène dans le mélangeur dans un état où le polyéthylène encapsule la charge inorganique.

11. Procédé selon la revendication 10, où la charge inorganique est le calcaire broyé.

12. Procédé selon la revendication 10, où la charge inorganique est l'ardoise.

13. Procédé selon la revendication 10, où la charge inorganique est le schiste.

14. Procédé selon la revendication 10, où la création comprend également : le moulage d'au moins une face du bardeau de toiture composite pour simuler un tavaillon.

15. Procédé selon la revendication 10, où la création comprend également :
le moulage d'au moins une face du bardeau de toiture composite pour simuler une ardoise.

16. Procédé selon la revendication 10, où le bardeau de toiture composite a une épaisseur inférieure à un pouce, a une largeur entre environ 3 et 12 pouces, et a une longueur entre environ 6 et 24 pouces.
